

## UNITED STATES PATENT OFFICE

JAMES IVOR MORGAN JONES AND WILLIAM KILBY, OF LANCASTER, ENGLAND,  
ASSIGNORS TO SCOTTISH DYES, LIMITED, OF GRANGEMOUTH, SCOTLAND

## DYEING AND PRINTING

No Drawing. Application filed June 27, 1927, Serial No. 201,959, and in Great Britain June 28, 1926.

This invention relates to the production of dyed products and more especially to the use of soluble ester derivatives of reduced vat dyestuffs which eliminate the use of vats in the dyeing of textile fibres, that is the use of hydro-sulphite vats or strongly alkaline reducing liquors, such as may be prepared for example according to the processes described in British specifications Nos. 186, 55 057, 202,630, 202,632, 231,889, 245,587, 247, 787, 248,802, 251,491, 258,626, 260,638, 260, 647, 261,139 and 263,898.

The object of the invention is primarily to provide an improvement or modification in connection with these processes.

The invention consists in a process for the production of dyed products by means of soluble ester derivatives of reduced vat dyestuffs which eliminate the use of vats according to which process dyeing is effected by padding and the material is steamed without drying after the padding process, the steamed material being subsequently entered into a development bath.

The invention also consists in a process which comprises the padding of soluble ester derivatives of leuco vat dyestuffs on to textile fibres, particularly such derivatives as may be prepared by processes of the kind indicated in the specifications referred to above, together with an oxidizing agent which is substantially inactive under the conditions of steaming, then freeing the padded goods from superfluous liquor and without drying, steaming the goods, treating them in a developing bath, rinsing and, if desired, soaping.

The invention also consists in a modification of the process according to the preceding paragraph in which an acid oxidizing agent is added to the developing bath instead of to the padding bath.

The invention further consists in a process as indicated in any of the preceding three paragraphs which includes the employment in the process of emulsifying or dispersing agents such as soluble oil or the like, soda ash or other weak alkali or Monopole soap, either as an addition to the padding liquor or by

treating therewith cloth or the like which is to be padded.

The invention further consists in processes for the dyeing of materials substantially as hereinafter described and in dyed products when prepared by those processes or by the obvious chemical equivalents thereof.

The following examples illustrate how the invention may be carried into effect, all parts being parts by weight:

## Example 1

The cloth is padded on a padding mangle at 95° C. with a solution made as follows:

|                                       | Parts by weight |
|---------------------------------------|-----------------|
| Soledon jade green (commercial paste) | 10-50           |
| Sodium nitrite                        | 1               |
| 6% gum dragon thickening              | 8               |
| Soluble oil                           | 70              |
| Water to                              | 1               |
|                                       | 100             |

After removal of superfluous liquor it is then steamed without drying for 10 minutes in an ordinary Mather & Platt steamer, and developed in an open width soaping machine by passing through 1 per cent. sulphuric acid, then rinsing and soaping.

## Example 2

The cloth is padded on a padding mangle at 95° C. with a solution made up as follows:

|                          | Parts by weight |
|--------------------------|-----------------|
| Soledon yellow           | 10              |
| 6% gum dragon thickening | 8               |
| Soda ash                 | 1               |
| Water up to              | 96              |
|                          | 100             |

It is then steamed without drying for 10 minutes in an ordinary Mather & Platt steamer and developed in an open width soaping machine by passing through 1 per cent. sulphuric acid containing 1 per cent. of bichromate of soda at 70° C. then rinsing and soaping.

*Example 3*

The cloth is padded on a padding mangle at 85° C. with a solution made as follows:—

|                          | Parts by weight |
|--------------------------|-----------------|
| 5 Indigosol pink HR      | 5               |
| 6% gum dragon thickening | 5               |
| Soluble oil              | 2               |
| Sodium nitrite           | 1               |
| 10 Water to              | 100             |

It is finally treated as in Example 1.

*Example 4*

15 The cloth is padded on a padding mangle at 45° C. with a solution made up of:—

|                          | Parts by weight |
|--------------------------|-----------------|
| 20 Indigosol 04B         | 5               |
| 6% gum dragon thickening | 5               |
| Soluble oil              | 2               |
| Sodium nitrite           | 1               |
| 25 Water up to           | 100             |

The cloth is then steamed without drying and developed as in Example 1.

*Example 5*

30 This is an example illustrating the variation of proportions of soluble oil or the like which may conveniently be used in comparison with the concentration of dyestuff in the padding liquor.

35 The cloth is padded on a padding mangle at temperatures of about 90–95° C. with one or other of the following solutions:—

|                             |     |     |      |     |     |     |       |
|-----------------------------|-----|-----|------|-----|-----|-----|-------|
| Dyestuff paste              | 50  | 100 | 200  | 300 | 400 | 500 | parts |
| Soluble oil                 | 7.5 | 10  | 12.5 | 15  | 20  | 25  | parts |
| Sodium nitrite              | 10  | 10  | 10   | 10  | 10  | 10  | parts |
| 40 6% gum dragon thickening | 8   | 8   | 8    | 8   | 8   | 8   | parts |

Water to 1000, 1000, 1000, 1000, 1000, 1000

The cloth is then steamed without drying and the colour developed as in Example 1.

*General*

Since the products referred to as used for dyeing are comparatively new, the following 50 information is given concerning them:—

(a) Soledon jade green (Scottish Dyes, Limited) appears to be a sodium salt of a sulphuric acid ester prepared from Caledon jade green (colour index 1101.)

55 (b) Soledon yellow (Scottish Dyes, Limited) is apparently the sodium salt of a sulphuric acid ester prepared from Caledon yellow G. (colour index 1118.)

(c) Indigosol pink HR. (Durand and Huguenin) is probably a sulphuric acid ester prepared from Helindone pink R. (colour index, commercial name index).

(d) Indigosol 4B (Durand and Huguenin) is probably the disulphuric acid ester of 60 indigo MLB/4B. (colour index 1184).

Having now described our invention, what we claim as new and desire to secure by Letters Patent is:—

1. The process which comprises the padding of soluble ester derivatives of leuco vat dyestuffs on to textile fibres together with an oxidizing agent which is substantially inactive under the conditions of steaming, then freeing the padded goods from superfluous liquor and next without drying, steaming the goods subsequently treating them in a developing bath and rinsing.

2. A process for the production of dyed products by means of soluble ester derivatives of reduced vat dyestuffs which eliminate the use of vats which consists in padding the aforesaid derivatives on to the material to be dyed, steaming the material without an intermediate drying stage and subsequently developing the colour on the steamed material.

3. A process as claimed in claim 2 which consists in carrying into effect the padding process in the presence of a dispersing agent.

In testimony whereof we have signed our names to this specification.

JAMES IVOR MORGAN JONES.  
WILLIAM KILBY.

70

75

80

85

90

95

100

105

110

115

120

125

130